

## [54] MECHANICAL SHAPING

[75] Inventors: **Jack M. Beigay, Freeport; Edward G. Chobey, Jr., Pittsburgh, both of Pa.; Joseph S. Kaferle, Ashtabula, Ohio**

[73] Assignee: **Allegheny Ludlum Industries, Inc., Pittsburgh, Pa.**

[22] Filed: **Mar. 10, 1972**

[21] Appl. No.: **233,783**

**Related U.S. Application Data**

[63] Continuation-in-part of Ser. No. 25,589, April 3, 1970, abandoned.

[52] **U.S. Cl. .... 72/46**

[51] **Int. Cl. .... B21c 3/14, B21c 23/24, B21j 3/00**

[58] **Field of Search...252/12, 12.2, 12.4, 12.6, 252/52 R, 56 S; 72/41, 42, 43, 46, 47, 286, 289**

[56] **References Cited****UNITED STATES PATENTS**

3,456,469 7/1969 Clappier et al. .... 252/12

|           |         |                       |          |
|-----------|---------|-----------------------|----------|
| 3,453,208 | 7/1969  | Gallagher et al. .... | 252/12   |
| 2,135,659 | 11/1938 | Elfstrom ....         | 72/43    |
| 2,346,124 | 4/1944  | Dew ....              | 252/52 R |
| 3,031,749 | 5/1962  | Adams ....            | 252/52 R |

**FOREIGN PATENTS OR APPLICATIONS**

1,004,836 9/1965 Great Britain .... 72/46

*Primary Examiner—Charles W. Lanham*

*Assistant Examiner—E. M. Combs*

*Attorney, Agent, or Firm—Vincent G. Giola*

[57] **ABSTRACT**

A method of mechanically shaping a metallic object, which comprises the steps of, coating a metallic object with a ductile, polyvinyl acetate and/or polyvinyl alcohol, non-metallic polymer base material having a maximum thickness of 0.1 mil, and increasing the length of the coated metallic object while simultaneously reducing its cross-sectional area with a former which substantially surrounds its perimeter.

**18 Claims, No Drawings**

## MECHANICAL SHAPING

This application is a continuation-in-part of now abandoned copending application Ser. No. 25,589 filed April 3, 1970.

The present invention relates to an improved method for mechanically shaping an object and more particularly to an improved method for mechanically shaping a metallic object.

Copper plating has been applied to carbon steel golf shafts prior to mechanical shaping. It provides a coating which furnishes the steel with protection against scratching and marking and provides the steel with a surface which holds, retains, and carries lubricants into close tolerance formers, i.e., mechanical shapers.

A similar use of copper plating on stainless steel golf shafts has not, however, proved to be desirable. The adhesion of copper onto stainless steel is not as dependable or as strong as is the adhesion of copper onto carbon steel. Copper plated stainless steel often results in the need for replating or in the flaking off of copper during shaping.

With the use of copper plating on stainless steel golf shafts all but ruled out, there arose a need for a protective coating which could be used in those mechanical shaping operations wherein a metallic object, e.g., a golf shaft, is passed through a former which substantially reduces the cross-sectional area of the object. The coating had to furnish the stainless steel with protection against scratching and marking and had to provide the steel with a surface which holds, retains, and carries lubricants.

We have found that polyvinyl acetate and polyvinyl alcohol, non-metallic polymer base coatings, having a maximum thickness of 0.1 mil, can be used on stainless steel golf shafts and other metallic objects to provide the protection that copper plate furnishes carbon steel golf shafts. Coatings of this general nature have been used for protection of surfaces which undergo normal handling and long-time storage, but have not been successfully used in mechanical shaping operations wherein a metallic object is placed between or passed through a former which substantially surrounds its perimeter. Mechanical shaping operations of this nature produce sizeable reductions in area and subject an object to a type of treatment which is not encountered during normal handling and even during other forms of mechanical shaping, such as rolling and deep drawing. Rolling and deep drawing do not place the entire perimeter of the object being shaped in compression as does a former when an object is placed between or passed through it. Furthermore, formers which substantially surround the perimeter are prone to defects which scratch the object being formed and cannot be flooded with lubricants, as are roll formers.

British Patent Specification No. 1,004,836 discloses the use of polyvinyl acetate on metal surfaces which are being drawn, but states that polyvinyl acetate is a decidedly inferior coating, and the worst coating in a group of poor coatings. Significantly, the polyvinyl acetate was applied in a thickness of 0.35 mil whereas the maximum thickness of the present invention is 0.1 mil.

Still, an additional advantage which is not obtained from the use of copper plate is realized from the use of non-metallic polymer base coatings, when the shaped object is subsequently heat treated. Copper must be chemically or electrochemically stripped from the me-

chanically shaped objects prior to heat treatment. The non-metallic polymer base coatings, however, do not have to be removed. They can be left on the shaped object and are useful in reducing the amount of scale formed during heat treatment. This in turn minimizes the pickling which must be performed to remove scale and reduce the criticalities involved in pickling golf shafts and other objects which require close control of weight loss.

Use of the non-metallic polymer base coatings have still further advantages. First of all, the life of the former is increased as metal to metal contact is avoided. Secondly, the coatings can be left on the shaped object to provide protection during subsequent fabricating operations, e.g., wire coiling.

It is accordingly an object of this invention to provide an improved method of mechanically shaping a metallic object.

It is another object of this invention to provide an improved method of mechanically shaping and heat treating a metallic object.

It is a further object of this invention to provide an improved method of mechanically shaping and fabricating a metallic object.

25 The method of the present invention comprises the steps of coating a metallic object with a ductile, polyvinyl acetate and/or polyvinyl alcohol, non-metallic polymer base material which has a greater adherence to the metallic object than to itself and which has a surface which holds, retains, and carries lubricants into close tolerance formers, and increasing the length of the coated metallic object while simultaneously reducing its cross-sectional area with a former which substantially surrounds its perimeter. The coating must be ductile since the mechanically shaped article has more surface area after shaping than before, must have a greater adherence to the metallic object than to itself, i.e., it should crack before peeling, so that it will exhibit strong and dependable adhesion, and must have a surface which holds, retains, and carries lubricant through close tolerance formers, (numerous coatings would be wiped clean of lubricant upon entrance into a die) so as to facilitate shaping. The mechanical shaping operation could be drawing, pressing, extrusion swaging or

40 any other operations which encompasses the placing between or passing of a metallic object through a former. It generally causes a reduction in area of at least 20 percent, i.e., the cross-sectional area of the shaped object is generally less than 80 percent of the original cross-sectional area, from one or more passes through the former.

In certain instances the method encompasses a heat treating operation subsequent to shaping, e.g., stainless steel golf shafts are annealed and age hardened. Use of non-metallic polymer base materials is particularly desirable in these instances as they reduce the amount of scale formed during heat treating and in turn minimize pickling. As discussed above, this reduction in pickling is highly advantageous for the manufacture of golf shafts and other objects which require a control of weight loss. It should, however, be noted that it is often desirable to remove the lubricant from the coating by vapor degreasing or other treatment prior to heat treatment as many lubricants will soften the coating, thereby, reducing its effectiveness.

In other instances the method encompasses additional fabricating operations subsequent to the, herein-

before, described mechanical shaping operation in which the cross-sectional area of the object is reduced. These operations include coiling processes in which previously drawn stainless steel wire is wound into a spring by means of a coiling tool. During coiling the non-metallic polymer base coating protects the stainless steel from damage caused by coiling tools which would otherwise scratch and roughen the surface of the steel and, thereby decrease its corrosion resistance.

The method of this invention is believed to be applicable to a wide variety of metals and objects which can have various forms. Emphasis has been placed upon stainless steel as it is probably the most important decorative metal and one of the few that will retain its brilliant surface through the years. The only restriction placed upon the form of the metal object is that it be suitable for the particular shaping operations embraced by this invention. Wire, rods, tubes and bars are typical forms. Tubes are generally reduced with the aid of a mandrel to insure constant wall thickness.

Any of the well-known coating methods can be employed. The invention is not dependent upon the use of any particular coating method. Illustrative coating methods are dip coating, flow coating, spray coating, and roll coating.

The preferred coating solution which satisfies the requirements of this invention is an aqueous of polyvinyl acetate. The solution should contain at least 1 percent by weight, polyvinyl acetate to insure a coating of adequate thickness and preferably should contain at least 3 percent. An upper preferred limit of 15 percent, by weight, polyvinyl acetate is imposed as thicker coatings to not adhere as tenaciously as do thinner coatings and since thicker coatings are more difficult to remove. Solutions with more than 15 percent polyvinyl acetate are, however, within the scope of the invention as long as they do not yield a coating greater than 0.1 mil thick. Coatings thicker than 0.1 of a mil produce an excessive degree of chatter during mechanical shaping. Chatter is defined as vibrations of the former or workpiece which produce a wavy surface on the object being formed. Although we do not know for sure why coatings thicker than 0.1 mil affect the degree of chatter, we hypothesize that the use of thicker coatings results in a coating build-up at the entrance of the former and this in turn causes an irregular movement of the workpiece through the former. As stated above, the coatings of this invention have a greater adherence to the metallic object than to themselves and, moreover, thicker coatings do not adhere as tenaciously as do thinner coatings.

Polyvinyl alcohols are additional coating solutions which satisfy the requirements of this invention. They can be obtained by the transesterification of polyvinyl acetate with methyl alcohol under the action of acid or base catalysis. Methyl acetate is removed from the reaction mixture as a by-product. The polyvinyl alcohols can contain acetate groups which have not been transformed. Mixed polyvinyl alcohol-acetate resins will have properties intermediate between polyvinyl acetate and polyvinyl alcohol.

A wetting agent can be added to the coating solution to insure the best possible wetting action at the metal surface. The use of wetting agents is optional and by no means necessary. A fatty acid amino type of soap has been successfully used with aqueous solutions of poly-

vinyl acetate in ranges varying between 10-20 percent, by weight, of the total solids within the solution.

The following examples emphasize several aspects of the invention.

#### EXAMPLE I

A group of stainless steel golf shafts were dip coated in an aqueous solution of polyvinyl acetate which had a fatty amino type of soap present as an emulsifier. The 10 solids were approximately 7.5 percent by weight of the aqueous solution. A second group of golf shafts were dip coated in another aqueous solution of polyvinyl acetate which also had a fatty acid amino type of soap present as an emulsifier. The solids present in this solution 15 were approximately 5.55 percent by weight of the aqueous solution. Both groups of golf shafts were step tapered in a hydraulic press, age hardened at 900° F for 8 hours and subsequently pickled.

The shafts were substantially free from scratches and 20 marks and were of the proper weight.

#### EXAMPLE II

Stainless steel wires were coated with polyvinyl acetate coatings ranging from 0.067 to 0.4 mil in thickness, and subsequently drawn from a diameter of 0.101 inch to a diameter of 0.032 inch. The degree of chatter was recorded at various stages during drawing by rating the chatter on a scale of 0-5, with 5 being the highest degree thereof. The results of the tests are as follows:

| Size  | Coating Thickness (mils): |      |      |     |       |
|-------|---------------------------|------|------|-----|-------|
|       | 0.4                       | 0.27 | 0.13 | 0.1 | 0.067 |
| 0.089 | 5                         | 2    | 0    | 0   | 0     |
| 0.079 | 2                         | 2    | 0    | 0   | 0     |
| 0.072 | 0                         | 0    | 5    | 0   | 0     |
| 0.065 | 2                         | 2    | 0    | 0   | 0     |
| 0.058 | 1                         | 2    | 0    | 0   | 0     |
| 0.052 | 4                         | 1    | 3    | 0   | 0     |
| 0.047 | 3                         | 3    | 2    | 2   | 0     |
| 0.043 | 3                         | 5    | 3    | 2   | 0     |
| 0.038 | 2                         | 2    | 3    | 0   | 0     |
| 0.034 | 3                         | 1    | 2    | 0   | 0     |
| 0.032 | 3                         | 0    | 0    | 0   | 0     |
| Total |                           | 28   | 20   | 18  | 4     |

The test results stress the criticality of a maximum coating thickness of 0.1 mil. They show that chatter is virtually eliminated with a coating of 0.067 mil and eliminated for all practical purposes with a coating of 0.1 mil, and that chatter significantly increases with coating thicknesses in excess of 0.1 mil.

It will be apparent to those skilled in the art that the novel principles of the invention disclosed herein in connection with specific examples thereof, will suggest various other modifications and applications of the same. It is accordingly desired that in construing the breadth of the appended claims they shall not be limited to the specific examples of the invention disclosed herein.

We claim:

1. An improved method of mechanically shaping a metallic object, which comprises the steps of: coating said metallic object with a ductile, non-metallic polymer base material from the group consisting of polyvinyl acetate solutions, polyvinyl alcohol solutions and mixtures thereof, said polymer base material having a greater adherence to said metallic object than to itself and having a surface which holds, retains, and carries lubricants into close tolerance formers, said coating having a maximum thickness of 0.1 mil; and increasing the length of said coated metallic object while simulta-

neously reducing its cross-sectional area with a former which substantially surrounds its perimeter.

2. A method according to claim 1 wherein the step of increasing the length of said coated metallic object while simultaneously reducing its cross-sectional area comprises the step of drawing said object through said former.

3. A method according to claim 1 wherein the step of increasing the length of said coated metallic object while simultaneously reducing its cross-sectional area comprises the step of extruding said object through said former.

4. A method according to claim 1 wherein the step of increasing the length of said coated metallic object while simultaneously reducing its cross-sectional area comprises the step of pressing said object with said former.

5. A method according to claim 1 wherein the step of increasing the length of said coated metallic object while simultaneously reducing its cross-sectional area comprises the step of swaging said object with said former.

6. A method according to claim 1 wherein said metallic object is a stainless steel object.

7. A method according to claim 1 wherein said metallic object has a substantially circular perimeter.

8. A method according to claim 1 wherein the cross-sectional area of said metallic object is reduced at least 20 percent by said former.

9. A method according to claim 1 including the steps of heat treating said coated and mechanically shaped

metallic object and subsequently removing said coating therefrom.

10. A method according to claim 9 including the step of removing lubricant from the mechanically shaped object prior to heat treating.

11. A method according to claim 1 wherein said non-metallic polymer base material is an aqueous solution of polyvinyl acetate.

12. A method according to claim 11 wherein said aqueous solution of polyvinyl acetate contains at least about 1 percent by weight polyvinyl acetate.

13. A method according to claim 12 wherein said aqueous solution of polyvinyl acetate contains from about 3 percent to about 15 percent by weight polyvinyl acetate.

14. A method according to claim 13 wherein said aqueous solution of polyvinyl acetate contains a wetting agent.

15. A method according to claim 14 wherein said wetting agent is a fatty acid amino type of soap.

16. A method according to claim 1 wherein said non-metallic polymer base material is a polyvinyl alcohol.

17. A method according to claim 7 wherein said metallic object is a rod, wherein the step of increasing the length of said coated metallic object while simultaneously reducing its cross-sectional area comprises the step of drawing said rod into wire, and including the step of coiling said wire.

18. A method according to claim 17 wherein said metallic object is a stainless steel rod.

\* \* \* \* \*